

E. J. LOVEGROVE & N. G. CROMPTON,  
E. G. CROMPTON, EXECUTRIX OF N. G. CROMPTON, DEC'D.  
PAVING MATERIAL.  
APPLICATION FILED MAR. 2, 1915.

1,237,920.

Patented Aug. 21, 1917.



Witnesses.

Jesse B. Heller  
John M. Corrigan

Inventors

Edwin J. Lovegrove  
Nigel G. Crompton  
by Beaureve, Polymer, Lander

Atty.

# UNITED STATES PATENT OFFICE.

EDWIN JAMES LOVEGROVE AND NIGEL GEORGE CROMPTON, OF LONDON, ENGLAND;  
ELIZABETH GERTRUDE CROMPTON EXECUTRIX OF SAID NIGEL GEORGE CROMPTON,  
DECEASED; SAID EXECUTRIX ASSIGNOR TO SAID LOVEGROVE.

## PAVING MATERIAL.

1,237,920.

Specification of Letters Patent. Patented Aug. 21, 1917.

Application filed March 2, 1915. Serial No. 11,581.

*To all whom it may concern:*

Be it known that we, EDWIN JAMES LOVEGROVE and NIGEL GEORGE CROMPTON, subjects of the King of England, both residing 5 in London, England, have invented certain new and useful Improvements in Paving Material, of which the following is a specification.

This invention is for improvements in or 10 relating to paving material of the kind commonly known as manufactured asphalt, which consists generally of finely-divided material such as sand or the like and bituminous binding or setting material.

15 The present invention only has reference to a material which of itself alone will constitute a traffic-resisting surface. That is to say, it may be formed to any desired thickness (for example one or more inches) and 20 consolidated, as distinct from a dust-laying coat or a grouting for other paving materials such as macadam or the like. A grouting has previously been proposed consisting of approximately equal proportions 25 of purified tar or pitch and retorted shale or residue or ash of shale that has been treated in a retort or the like or calcined coal or the residue or ash of coal reduced to a fine impalpable powder. Such a composition 30 cannot, of itself, constitute a paving material contemplated by the present invention.

According to the present invention our 35 paving material consists solely of clinker or ash or like residue of combustion from a refuse destructor or incinerator, in a finely divided condition admixed, with a maximum of 20% of its weight of bituminous material.

40 Throughout the specification and claims wherever the term "refuse destructor residue" is employed, it is to be understood as indicating all forms of vitrified clinker or ash or like residue of combustion from a 45 refuse destructor or incinerator, other than coal or coke clinker or ash.

The invention also includes the paving material before or after it has been laid.

One feature of the invention consists in 50 the utilization of heat contained in the waste gases from the destructor furnace for wholly or partially drying or heating, or for wholly or partially drying and heating

the ingredients prior to, during or subsequently to their admixture.

55

In a preferred method of preparing an asphalt or paving material according to the present invention, the clinker, ash or the like is derived from a refuse destructor and is ground in an ordinary revolving mill or 60 breaker or other suitable grinding or pulverizing apparatus and which will break up into particles of angular form. The clinker or ash may be passed through the apparatus in an initially hot condition after removal 65 from the destructor or alternatively it may be taken in a cold condition. After grinding, the material is screened through a small mesh screen and is thence conveyed to driers heated by waste gases from the destructor 70 furnace. The heated and dried material may be further sifted or separated and stored in bins until required for mixing or it may be conveyed direct to the mixers, 75 where it is mixed with bituminous material.

The fine material obtained from the screening operation is mixed with about 10-20% of its weight of bitumen which may be either native bitumen, or bituminous residuum of asphaltic oils, sometimes called petroleum pitch. The bituminous material is preferably preliminarily heated by heat from the destructor gases before passing 80 into the mixing apparatus. The latter apparatus, however, may be heated during the 85 mixing operation also by the heat derived from destructor gases.

The material is removed from the mixing apparatus and is laid, while hot, in a loosened or powdered condition and consolidated (as for example by rolling or ramming) as an asphaltic layer or carpet one inch or thereabout in thickness, either on the surface of the road or path or upon a bituminous concrete, cement concrete or 90 some other prepared foundation. The ingredients may be conveniently mixed at a temperature from about 275°-375° F. while the mixture may be laid at a temperature 95 from about 250°-350° F.

100 It will be seen, therefore, that the products of refuse-destructors are utilized to advantage both in the supply of material and of heat. In addition to the heating of the various apparatus as above described, the 105 steam raised in the destructor boiler may be

employed to drive the necessary machinery. Such additional heat as may be necessary for the various apparatus employed (for example, the drier, mixer or heater for the 5 bituminous material) may be provided by external sources of heat.

The apparatus for drying and for mixing and heating the materials may be of any convenient construction and as there are 10 many forms of these apparatus available on the market, it is not necessary to describe them more fully herein. They may be heated either by the waste gases from the destructor alone or by steam generated by 15 heat from the destructor gases or by both these sources of heat together, or by heat from external sources or by any combination of these sources as may be convenient and requisite.

20 In a previously suggested paving composition destructor clinker has been screened to eliminate cinders, coke residues, breeze and fine material and the remainder, consisting only of hard vitrified material which 25 is not readily pulverizable, has been admixed with practically pure bituminous material and Portland cement. The latter ingredient is added to the mixture to fill up the interstices between the coarse particles 30 obtained from the specially sifted destructor clinker. It has also been proposed to form paving blocks consisting of 80% crushed clinker, 15% Trinidad or other asphalt and 5% of fine limestone or other 35 dust.

The vitrified destructor residue when crushed will break up into pieces of angular formation and can readily be separated when pulverized into a large number of 40 grades or degrees of fineness. Powdered stone and such like substances can ordinarily only be classified into three or four grades, whereas the destructor residue can be classified into about sixteen or eighteen 45 grades covering the same range of particles. As the material is broken up into pieces of angular formation it will more readily lock together into a solid mass with the bitumen binder, and as screened material 50 is formed from sixteen to eighteen different grades within the range of the usual screened material, it will pack together and consolidate in a much more satisfactory way than do other materials, and 55 therefore will provide a far better wearing surface than any material heretofore known.

A further advantage lies in the fact that the clinker may be used in a heated condition as it is removed from the furnace, 60 which obviates wholly or partially the necessity of subsequently heating it, or if it

is allowed to stand for some time after cooling, it can be conveniently stored so that the absorbed moisture does not assume so large a quantity as that contained in the 65 sand hitherto employed. Consequently less heat is required to dry it.

The accompanying drawing illustrates, in a purely diagrammatic fashion, the arrangements referred to herein. A grinding 70 apparatus is indicated at A driven from an engine A<sup>1</sup> which obtains its motive steam from the boiler of a dust-destroyer B. The material issuing from the grinder is screened through a mesh screen C and 75 thence it is taken to a drier D and driven by an engine D<sup>1</sup> which also obtains its steam from the boiler of the dust-destroyer. After the material has been dried it passes to a mixer E in which it is mixed with the 80 bituminous material, an engine E<sup>1</sup> obtaining its motive steam from the boiler of the dust-destroyer B driving the mixing vanes or the like. The drier D and the mixer E may be heated as is diagrammatically represented by hot gases obtained from the dust-destroyer and conveyed through pipes F to the two apparatus.

It will be understood that the drier need not necessarily have any mechanically moving parts but may be simply a heated receptacle and further such an apparatus may be eliminated altogether. Similarly, it is not necessary that the mixer be heated although it is preferable that it should be so.

95 Although details of the preparation and composition of a paving material have been specifically quoted above, the invention is not limited to those details as they may be varied according to the quality of the material required.

100 What we claim as our invention and desire to secure by Letters Patent is:—

1. A paving material consisting of pulverized refuse destructor residue of angular 105 formation and a bituminous binder.

2. A paving material consisting of pulverized refuse destructor residue of angular formation and 20 per cent. of its weight of 110 bituminous binder.

3. A paving material consisting of pulverized refuse destructor residue of angular formation and 10-20 per cent. of its weight of bituminous binder.

115 In testimony whereof we have signed our names to this specification in the presence of two subscribing witnesses.

EDWIN JAMES LOVEGROVE.  
NIGEL GEORGE CROMPTON.

Witnesses:

HAROLD WADE,  
HARRY I. KIRBY.